

# United States Patent [19]

Borbely et al.

[11] 3,983,018

[45] Sept. 28, 1976

[54] PURIFICATION OF NICKEL  
ELECTROLYTE BY ELECTROLYTIC  
OXIDATION

[75] Inventors: Gyula John Borbely, Copper Cliff;  
Alexander Illis, Mississauga;  
Bernardus Jacobus Brandt, Port  
Colborne, all of Canada

[73] Assignee: The International Nickel Company,  
Inc., New York, N.Y.

[22] Filed: Sept. 10, 1975

[21] Appl. No.: 612,011

[30] Foreign Application Priority Data

Feb. 12, 1975 Canada ..... 219948

[52] U.S. Cl. 204/130; 204/113

[51] Int. Cl.<sup>2</sup> C25F 7/02; C25D 21/16

[58] Field of Search 204/130, 149, 140, 232,  
204/112, 240, 113

[56] References Cited

UNITED STATES PATENTS

2,394,874 2/1946 Renzoni ..... 204/113

|           |        |                         |         |
|-----------|--------|-------------------------|---------|
| 3,334,034 | 8/1967 | Geldzahler.....         | 204/130 |
| 3,457,152 | 7/1969 | Maloney, Jr. et al..... | 204/130 |
| 3,640,805 | 2/1972 | Knight .....            | 204/130 |

FOREIGN PATENTS OR APPLICATIONS

|          |        |          |
|----------|--------|----------|
| S31-4904 | 6/1956 | Japan    |
| 185,072  | 7/1966 | U.S.S.R. |

Primary Examiner—T. M. Tufariello  
Attorney, Agent, or Firm—Walter A. Petersen; Ewan  
C. MacQueen; Raymond J. Kenny

[57] ABSTRACT

The presence of one or more of cobalt, iron, arsenic and lead is most substantially reduced in a nickel-containing electrolyte by an electrochemical process utilizing a high current density at the cathode in an electrolytic cell containing specific quantities of chlorides of alkali metals to form a fine nickel hydroxide precipitate. In a subsequent time dependent reaction under controlled pH conditions, nickel hydroxide reacts with the electrolyte to form insoluble precipitates of cobalt, iron, arsenic and lead which are removed from the electrolyte by filtration.

14 Claims, 1 Drawing Figure



FIG. 1.



## PURIFICATION OF NICKEL ELECTROLYTE BY ELECTROLYTIC OXIDATION

The present invention relates to the production of high purity nickel by electrorefining, and, more particularly, to an improved electrochemical process for markedly reducing the presence of cobalt, iron, arsenic and lead contaminants from the nickel-containing electrolyte.

During the electrorefining of nickel, it is usually necessary to purify the electrolyte by removing elements such as copper, cobalt, iron, arsenic and lead. In a currently used process described in Canadian Pat. No. 440,659, a high degree of electrolyte purification is accomplished, but this requires a number of complex stages to effect the removal of iron, copper and cobalt. The process of the present invention is deemed less costly, considered easier to carry forward and further differs in that electrochemical rather than chemical separation is used. Electrochemical techniques have been heretofore proposed. For example, in a prior art process, only cobalt was separated from nickel whereas in the present invention, iron, lead and arsenic are removed concurrent with the cobalt. The present invention eliminates the plating of metallic nickel at the cathode which presented a significant problem with the economic application of this prior art process. Further, the requirement for alkali additions necessary for control of pH is largely reduced through in situ generation of nickel hydroxide.

It has now been discovered that a nickel electrolyte used, for example, in the process of electrowinning nickel, can be purified prior to plating by an electrochemical means. The levels of the impurity elements cobalt, iron, arsenic and lead contained within the electrolyte can be reduced substantially. In the process of this invention, an impure nickel-containing electrolyte having low copper content and containing chloride salts of an alkali metal is introduced into an electrolytic tank containing one or more insoluble anodes and at least one cathode. The anode surface area is at least 20 times as great as the surface area of the cathode resulting in a high current density on the cathode surface. During electrolysis, nickel hydroxide and hydrogen form at the cathode. Elemental chlorine forms at the anode and immediately reacts with the electrolyte to form hydrochloric and hypochlorous acids. The latter serves as an oxidizer in a time-dependent reaction with cobalt.

Cobalt, iron, arsenic and lead precipitates begin to form in the electrolytic tank through preferential oxidation by the hypochlorous acid and precipitation is generally completed in a retention tank removed from the electrolytic tank. After a sufficient reaction period, the cobalt, iron, arsenic and lead precipitates are separated from the purified electrolyte by a conventional filtering operation.

It is an object of this invention to remove substantially at least one impurity from a group consisting of cobalt, iron, arsenic and lead from a nickel electrolyte.

It is a further object of this invention to reduce the quantity of raw materials and the amount of energy consumed in the purification of nickel electrolyte used in an electrorefining operation.

The foregoing objects and the means whereby they are attained will be more fully understood from the following description taken in conjunction with the

accompanying drawing in which there is shown a sectional view of the electrolytic and retention tanks.

Generally speaking, the process of this invention is used to remove at least one impurity from a group consisting of cobalt, iron, arsenic and lead from an aqueous, essentially copper-free, nickel-containing electrolyte and comprises immersing at least one anode and at least one cathode into said electrolyte, said electrolyte containing a chloride salt of an alkali metal; applying a current between said anode and said cathode for a time period sufficient to generate in said electrolyte an equivalent chlorine content of at least about 0.05 gram per liter while maintaining the current density at said cathode at a level sufficient to prevent substantial deposition of metal at said cathode but sufficient to generate a metal hydroxide in the vicinity of said cathode; increasing the pH of said electrolyte whereby said equivalent chlorine produced reacts with at least one impurity present in said electrolyte to provide a precipitate containing said at least one impurity; and separating said precipitate from said electrolyte.

It is a requirement of the process that the surface area of the anode be at least about 20 times that of the cathode. Due to this high surface area ratio, high current densities, between about 6,000 and about 39,000 amps./m<sup>2</sup> are attained on the surface of the cathode. High current density is required to avoid plating of nickel and other metallic ions at the cathode. Below about 6,000 amps./m<sup>2</sup> metallic ions will plate, and above about 39,000 amps./m<sup>2</sup> metallic ions and hydrates will plate on the cathode. The current density at the anode is limited by geometric considerations and the ability to efficiently generate and react chlorine with the electrolyte. That is, with decreasing anode surface area, greater amounts of chlorine will bubble off rather than dissolve and also a greater tendency for breakdown of newly formed hypochlorous acid will exist.

Successful operation of the process is dependent upon the presence of chloride ions of an alkali metal, preferably sodium. It is necessary that the chloride ion concentration be greater than about 5 grams per liter and the alkali metal concentration be greater than about 2 grams per liter. Upper limits have not been established for these ions however, substantial quantities may be present. For example, in the case of an "all-chloride" bath, as much as about 150 gpl of chloride ion may be present.

The anode material used in this invention may be graphite, or a metallic, acid-resistant, conductive material. The cathode material may be a steel in rod or other suitable form. Other electrode materials and forms may also be used and include conductive substances having sufficient corrosion resistance in oxidizing alkaline and acid environments. The spacing of anode and cathode is not considered critical, however, they should be placed within reasonable proximity to allow efficient operation yet apart a sufficient distance to provide separation of the electro-chemical reactions and to avoid short circuiting.

Referring to FIG. 1, electrolyte which has passed through a copper removal process and containing very little copper enters the agitated electrolytic tank 12 through pipe 11 where it interacts with the anode 13 and the cathode 14. A first addition tank 15 can be used to adjust the hydrogen ion concentration or pH of the electrolyte. The reactions at the anode and cathode are dependent on the presence of chloride salts of al-

kali metals and a high current density at the cathode. It is advantageous to insert a baffle 16 between the oxidized electrolyte and the exit pipe 17 to reduce the through-put of non-oxidized electrolyte.

The oxidizer formed at the anode, hypochlorous acid, begins to react with divalent cobalt ions and similar ions of iron, arsenic and lead in the electrolytic tank. However, since the oxidation reaction is time dependent, the solution is generally transferred through exit pipe 17 to a retention tank 18 generally by gravity feed.

The majority of the cobaltous ion to cobaltic oxide reaction occurs within the agitated retention tank. A controlled quantity of a pH adjusting liquid is introduced to the retention tank from a second addition tank 19 to adjust the hydrogen ion concentration or pH of the electrolyte. The retention tank contains a baffle 20 which causes separation of the incoming electrolyte from that which has already reacted. The oxidized electrolyte leaves the retention tank through pipe 21 and is pumped or gravity-fed to a filter not shown. Cobalt, iron, arsenic and lead precipitates are removed from the liquid stream in the filtering operation. Purified electrolyte may be returned to the refining circuit at this point or alternatively sent through one or more additional processing sequences as aforedescribed for further reduction of impurity content.

The operating temperature of the electrolytic and retention tanks is generally maintained at the same temperature as that of the nickel electrorefining circuit. Temperatures in the range of about 50°C. to about 65°C. are used.

All-sulfate or all-chloride electrolytes and mixtures of these may be purified with the process of this invention. The compositions in grams per liter of typical nickel electrolytes treated by this process follow:

|                               |        |                                |           |
|-------------------------------|--------|--------------------------------|-----------|
| Ni <sup>++</sup>              | 40-80  | H <sub>3</sub> BO <sub>3</sub> | 5-20      |
| Co <sup>++</sup>              | .05-.5 | As <sup>+++</sup>              | .001-.2   |
| Na <sup>+</sup>               | 2-50   | Pb <sup>++</sup>               | .0001-.01 |
| Cl <sup>-</sup>               | 5-90   | Cu <sup>++</sup>               | up to .01 |
| SO <sub>4</sub> <sup>2-</sup> | 2-150  |                                |           |

The chemical reactions believed to occur during electrochemical oxidation of the electrolyte will be considered in order to demonstrate the operation of this invention. The discussion will center on cobalt; however, similar reactions are believed to occur with the iron, arsenic and lead ions present in the solution.

Under the influence of the applied current, sodium or other alkali metal ions are attracted to and arrive at the cathode before nickel and other metallic ions due to their higher mobility. Sodium ions pick up electrons from the cathode and immediately react with water present in the electrolyte to form sodium hydroxide and hydrogen gas, the latter escaping from the electrolytic tank. Nickel ions encounter the increased concentration of sodium hydroxide in the vicinity of the cathode and react to form a fine nickel hydroxide precipitate which serves to beneficially increase the pH of the electrolyte at this stage as well as later on in the process. It is generally considered beneficial to thoroughly agitate the electrolyte to break up the nickel hydroxide precipitate into a fine dispersion suited for neutralization of acid. The pH of the electrolyte upon entering the electrolytic tank is about 2.5 to 5.5 for a batch

operation and from about 3.2 to 4.5 is preferred in a continuous operation.

Chloride ions give up electrons and form elemental chlorine at the anode. This chlorine immediately reacts with water contained in the electrolyte forming hypochlorous and hydrochloric acids. A summation of the reactions believed to occur during electrolysis follows:



The oxidizing power of the electrolyte at this point in the process is governed by the current density at the anode, efficiency of chlorine reaction with the electrolyte, tank size, and the residence time in the electrolytic cell. Typically, a concentration equivalent to about 0.2 to 0.8 grams per liter of chlorine is attained in this process. The residence time in the electrolytic tank is generally between about 2 and 20 minutes and the pH is in the range 3.6 to 4.2.

Hypochlorous acid is the ingredient essential to the oxidation of unwanted metallic ions. Precipitation of hydrated cobaltic oxide or cobaltic hydroxide as well as oxidic forms of iron, arsenic and lead begins within the electrolytic cell by reaction with the hypochlorous acid; however, the rate of reaction is relatively slow. Because of this, the liquid containing hypochlorous acid is generally transferred to a retention tank where it is held for sufficient time, from about 20 minutes to about 2 hours and typically 40 minutes, for the oxidation reaction and hydrolyzation to occur. It has been found expedient to add a small amount of an alkaline solution such as sodium carbonate solution to the electrolyte in the retention tank to raise its pH to at least 4.5 to as much as, for example, 5.0 from the previous 3.6 to 4.2 level.

A summation of the reactions that start in the electrolytic tank and proceed further in the retention tank are given by the following equation:



In a continuous production operation, however, it is advantageous to add a slurry of nickel carbonate to avoid an unnecessary increase in the sodium ion concentration of the electrolyte. A summation of the reactions believed to occur with this procedure follows:



The process as described is preferentially used for continuous production of refined nickel; however, a batch operation is also considered within the scope of this invention especially where high concentrations of cobalt are present, for example, 1 to 10 grams per liter.

Furthermore, by careful control of the oxidation potential and the pH of the electrolyte, it is possible to selectively precipitate unwanted elements and in this way a purer cobalt precipitate is obtained. This is advantageous to the process for recovery of this valuable metal.

The selective process involves two stages. In the first, the electrolyte is partially oxidized, adjusted to a pH slightly below that required for cobalt precipitation but high enough for precipitation of iron, arsenic and lead. After hydrolyzation, the iron, arsenic and lead precipi-

tates are removed by filtration. In the second stage, the electrolyte is fully oxidized in an electrolytic tank and the pH in the retention tank is increased sufficiently to precipitate cobalt of high purity since the electrolyte is substantially free from iron, arsenic and lead at this point.

The use of other halide salts, e.g., bromides and iodides, of alkali metals is also contemplated in this invention and may be substituted for the sodium chloride addition. However, sodium chloride is preferred in the operation of this invention due to its ready availability and low cost.

In order to give those skilled in the art a better understanding of the invention, the following illustrative examples are given which demonstrate the capabilities of the process for substantial removal of cobalt, iron, arsenic and lead from a copper-free nickel-containing electrolyte.

#### EXAMPLE 1

Tank house electrolyte containing 73.0 grams per liter (typically 40-80 gpl nickel), about 33-45 gpl sodium, 46-56 gpl chloride, 100-150 gpl sulfate, 13-16 gpl boric acid and less than 0.01 gpl of dissolved copper and having a pH of 2.9 was passed through an electrolytic tank of 1 liter capacity. The tank contained a stainless steel wire cathode, 2.4 mm diameter by 6.4 cm long, and 2 graphite anodes 1.3 cm  $\times$  6.4 cm  $\times$  9 cm. A direct current of 4 amperes was supplied for the electrolysis at a current density of 8,400 amps./m<sup>2</sup> at the cathode, 410 amps./m<sup>2</sup> at the anode with a cell voltage of 5.5 volts. The power consumption was 3.3 watt-hours/liter and the average residence time for the electrolyte in the electrolytic tank was 9 minutes. The temperature of the electrolytic and retention tanks was controlled between 54°C. and 60°C. in this and all of the examples to be compatible with the currently used nickel electrorefining process.

Upon leaving the electrolytic tank, the oxidizing power of the solution was equivalent to 0.290 grams per liter of chlorine. Table I shows the level of cobalt, iron and arsenic as well as the pH of the feed to the electrolytic tank. The concentration of these elements in the effluent was only slightly lowered. A 30 minute hold in the agitated retention tank reduced the cobalt content of the electrolyte by 90.7%, the iron content by 97.8% and the arsenic content by 95.0%. This required the addition of 1.0 grams per liter of sodium carbonate to the retention tank. The nickel to cobalt ratio in the filtered precipitate was 3.0.

TABLE I

| Electrolytic Oxidation of a Lead-Free Tank House Electrolyte |       |        |        |
|--------------------------------------------------------------|-------|--------|--------|
|                                                              | Co    | Fe     | As     |
| Electrolytic Tank Feed, gpl                                  | 0.150 | 0.047  | 0.014  |
| Electrolytic Tank Effluent, gpl                              | 0.140 | 0.020  | 0.007  |
| Filtrate after 30 min. in<br>Retention Tank, gpl             | 0.014 | <0.001 | 0.0007 |
|                                                              |       |        | pH     |
|                                                              |       |        | 2.9    |
|                                                              |       |        | 4.2    |
|                                                              |       |        | 4.5    |

#### EXAMPLE 2

In a test similar to that described in Example 1, a tank house electrolyte essentially free of copper and arsenic and containing 69.1 gpl of nickel and having a pH of 2.8 was subjected to electrolytic oxidation. Current density was 8,400 amps./m<sup>2</sup> at the cathode, 410 amps./m<sup>2</sup> at the anode and the cell voltage was 5.5 volts. The solution had a residence time of 10 minutes

in the electrolytic tank and the power consumption was 3.7 watt-hours per liter. The oxidizing power of the solution following this stage of the operation was equivalent to 0.457 gpl of chlorine. During the precipitation step, 1.5 gpl of sodium carbonate was added to the retention tank. As shown in Table II, after a 30-minute hold in the agitated retention tank and filtering, 97.7% of the cobalt, 99.2% of the iron and 93.6% of the lead were removed from the electrolyte. The ratio of nickel to cobalt in the precipitate was 1.2.

TABLE II

| Electrolytic Oxidation of an Arsenic-Free Tank House Electrolyte |       |        |        |     |
|------------------------------------------------------------------|-------|--------|--------|-----|
|                                                                  | Co    | Fe     | Pb     | pH  |
| Electrolytic Tank Feed, gpl                                      | 0.260 | 0.133  | 0.0047 | 2.8 |
| Electrolytic Tank Effluent, gpl                                  | 0.250 | 0.030  | 0.001  | 3.7 |
| Filtrate after 30 minutes in<br>Retention Tank, gpl              | 0.006 | <0.001 | 0.0003 | 4.5 |

#### EXAMPLE 3

A synthetic electrolyte free from copper, lead and arsenic and containing 60.0 gpl of nickel and having a pH of 2.9 was subjected to electrolytic oxidation in the equipment described in Example 1. Current Density was 8,400 amps./m<sup>2</sup> at the cathode, 410 amps./m<sup>2</sup> at the anode and the cell voltage was 5.5 volts. The solution had a residence time of 6 minutes in the electrolytic tank and the power consumption was 2.2 watt-hours per liter. The oxidizing power of the solution following this stage of the operation was equivalent to 0.204 gpl of chlorine. A total of 0.92 gpl of sodium carbonate was added to the retention tank during the precipitation step. As shown in Table III, after a 30-minute hold in the agitated retention tank and filtering, the cobalt concentration was reduced by 98.7% and the iron by 97.5%. The ratio of nickel to cobalt in the filtered precipitation was 1.7.

TABLE III

| Electrolytic Oxidation of an Arsenic- and Lead-Free Synthetic Electrolyte |       |        |     |  |
|---------------------------------------------------------------------------|-------|--------|-----|--|
|                                                                           | Co    | Fe     | pH  |  |
| Electrolytic Tank Feed, gpl                                               | 0.150 | 0.040  | 2.9 |  |
| Electrolytic Tank Effluent, gpl                                           | 0.145 | 0.025  | 4.1 |  |
| Filtrate after 30 minutes in<br>Retention Tank, gpl                       | 0.002 | <0.001 | 4.5 |  |

#### EXAMPLE 4

A two-stage electrolytic oxidation treatment was carried out which selectively removed iron and arsenic while occluding only small amounts of nickel and cobalt in the first stage. Second stage electrolytic oxidation removed cobalt as a hydrate.

Tank house electrolyte with a pH of 2.9 was electrolytically oxidized for about 3 minutes to a state equivalent to 0.093 grams per liter of chlorine using the equipment described in Example 1. Current density was 8,400 amps./m<sup>2</sup> at the cathode, 410 amps./m<sup>2</sup> at the anode and the cell voltage was 5.5 volts. By adjusting the pH to 4.0 with 0.47 gpl of sodium carbonate in the agitated retention tank and holding for 1 hour at 54°C., 94.7% of the iron, 98.6% of the arsenic and 39.0% of the lead were removed. Table IV shows the assay of the electrolyte for this and the other stages of the process.

The solution was then brought to a state equivalent to 0.61 gpl of chlorine by electrolytically oxidizing for about 9 minutes using the aforescribed current densities and voltage. By adjustment of the pH to 4.5, again through the addition of 1.0 gpl of sodium carbonate, 5

Table V shows that as the sodium ion concentration was increased, the final pH increased and, more importantly, that metallic nickel stopped forming upon the cathode when the pH in the electrolytic tank rises above the solution starting pH of 3.1.

TABLE V

| NA+ Concentration<br>grams/liter | Alkali Metal Ion Concentration |                                                 |                                          |
|----------------------------------|--------------------------------|-------------------------------------------------|------------------------------------------|
|                                  | Final Tank<br>pH               | Cathode Deposit after 9 minutes<br>at 4 amperes | Composition                              |
| 0.0                              | 2.05                           | 550                                             | Metallic Ni                              |
| 0.5                              | 2.40                           | 470                                             | Metallic Ni + Trace of $\text{Ni(OH)}_2$ |
| 1.0                              | 2.70                           | 230                                             | Metallic Ni + $\text{Ni(OH)}_2$          |
| 1.5                              | 3.10                           | 160                                             | $\text{Ni(OH)}_2$ + Metallic Ni          |
| 2.0                              | 4.20                           | 20                                              | $\text{Ni(OH)}_2$ + Trace Metallic Ni    |
| 5.0                              | 4.35                           | 18                                              | $\text{Ni(OH)}_2$ only                   |
| 10.0                             | 4.55                           | 17                                              | $\text{Ni(OH)}_2$ only                   |
| 15.0                             | 4.48                           | 13                                              | $\text{Ni(OH)}_2$ only                   |
| 25.0                             | 4.61                           | 10                                              | $\text{Ni(OH)}_2$ only                   |
| 40.0                             | 4.52                           | 10                                              | $\text{Ni(OH)}_2$ only                   |

and holding for one hour in the agitated retention tank, 25 98.5% of the cobalt was removed as a hydrate having a nickel to cobalt ratio of 1.4. An additional 4.8% of the iron was removed during this stage bringing the total for iron to 99.5% removed. Also, 56.8% more lead was removed at this point bringing the total percentage of lead removed to 95.8%. This selective removal process for iron, arsenic and lead followed by cobalt offers considerable advantage in later processing for recovery of cobalt from the precipitate.

TABLE IV

| Two-Stage Electrolytic Oxidation |       |        |         |         |
|----------------------------------|-------|--------|---------|---------|
|                                  | Co    | Fe     | Pb      | As      |
| Starting Electrolyte, gpl        | 0.26  | 0.133  | 0.0059  | 0.0045  |
| Filtrate 1, gpl                  | 0.26  | 0.007  | 0.0036  | 0.00006 |
| Filtrate 2, gpl                  | 0.004 | 0.0006 | 0.00025 | 0.00006 |

EXAMPLE 5

35 40

## EXAMPLE 6

Controlling the pH of the electrolyte entering the electrolytic tank is important to the efficiency with which impurities can be removed. A tank-house electrolyte containing 69.0 gpl of nickel, 0.260 gpl of cobalt, 0.006 gpl of lead, 0.0045 gpl arsenic and 0.133 gpl of iron was introduced to an electrolytic tank as described in Example 1. Upon entering this tank, the pH was continuously adjusted by addition of sodium carbonate solution from a first addition tank so that constant values ranging from pH 2.7 to 5.2 were attained. The cathode current density was generally about 16,800 amps./m<sup>2</sup> and the oxidizing power of the electrolyte was equivalent to about 0.85 gpl of chlorine. As shown in Table VI, the efficiency of cobalt removal was increased from 88.5% to 98.8% while the efficiency of lead, arsenic and iron removal remained constant. This improvement however, is offset by an increase in the quantity of nickel co-precipitated with the cobalt.

TABLE VI

|                                                 | Effect of Electrolyte pH on Impurity Removal |        |        |        |        |
|-------------------------------------------------|----------------------------------------------|--------|--------|--------|--------|
|                                                 | 1                                            | 2      | 3      | 4      | 5      |
| Electrolyte Feed pH                             | 2.7                                          | 3.2    | 3.7    | 4.7    | 5.2    |
| Electrolyte Effluent pH                         | 3.8                                          | 3.9    | 4.1    | 4.2    | 4.2    |
| Cathode Current Density<br>amps./m <sup>2</sup> | 16,800                                       | 12,600 | 16,800 | 16,800 | 16,800 |
| Electrolytic Tank Voltage                       | 9.0                                          | 7.0    | 9.0    | 9.0    | 9.0    |
| Chlorine Generation gpl                         | 0.87                                         | 0.85   | 0.82   | 0.80   | 0.90   |
| Final Cobalt Content gpl                        | 0.030                                        | 0.012  | 0.016  | 0.012  | 0.003  |
| Removal Efficiency, %                           |                                              |        |        |        |        |
| Co                                              | 88.5                                         | 95.4   | 93.8   | 95.4   | 98.8   |
| Pb                                              | 98.3                                         | 98.3   | 98.3   | 98.3   | 98.3   |
| Fe                                              | 98.5                                         | 98.5   | 98.5   | 98.5   | 99.6   |
| As                                              | 98.6                                         | 98.6   | 98.6   | 98.6   | 98.6   |
| Ratio Ni:Co in Precipitate                      | 1.9                                          | 2.7    | 3.1    | 3.5    | 4.0    |

The minimum requirement for alkali metal ion was 60 established by adding increasing amounts of sodium in the form of sodium sulfate to an electrolyte containing 0.068 gpl of sodium, 60.6 gpl of nickel, 36.6 gpl of chloride ion, 49.6 gpl of sulfate ion and 16 gpl of boric acid. The equipment used was the same as that previously described in Example 1. The cathode current density was 8,400 amps./m<sup>2</sup> and the pH of the solution was initially 3.1.

65

## EXAMPLE 7

Utilization of the metal hydroxide generated in the electrolytic oxidation process is an important feature since it reduces the amount of alkali required for precipitation of impurities. The results contained in Table VII show the amount of alkali required to precipitate the impurities with and without the use of electrolytic oxidation for the purification of the tank house electrolyte described previously in Example 2.

TABLE VII

Materials and Power Consumed During Electrolytic Oxidation

|                                | cobalt removal<br>gpl | Na <sub>2</sub> CO <sub>3</sub><br>equivalent<br>gpl | chlorine<br>gpl | power<br>watt-<br>hours/<br>liter |
|--------------------------------|-----------------------|------------------------------------------------------|-----------------|-----------------------------------|
| Without electrolytic oxidation | 0.244                 | 2.74                                                 | 0.085           | nil                               |
| With electrolytic oxidation    | 0.254                 | 1.50                                                 | nil             | 3.7                               |

The soda ash equivalent is 1.24 grams/liter less for the electrolytic oxidation process than for the presently used process. The consumption of 45% less alkali coupled with in situ generation of chlorine represents a considerable savings in raw materials and indirectly, in power requirements.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. A process for removing at least one impurity from a group consisting of cobalt, iron, arsenic and lead from an aqueous, essentially copper-free, nickel-containing electrolyte which comprises: immersing at least one anode and at least one cathode into said electrolyte, said electrolyte containing a chloride salt of an alkali metal; applying current between said anode and said cathode for a time period sufficient to generate in said electrolyte an equivalent chlorine content of at least about 0.05 gram per liter while maintaining the current density at said cathode at a level sufficient to prevent substantial deposition of metal at said cathode but sufficient to generate a metal hydroxide in the vicinity of said cathode; increasing the pH of said electrolyte whereby said equivalent chlorine produced reacts with at least one impurity present in said electrolyte to provide a precipitate containing said at least one impurity; and separating said precipitate from said electrolyte.

2. A process as defined in claim 1, wherein the total surface area of said anode is at least 20 times the surface area of said cathode.

3. A process as defined in claim 1, wherein a current density of 6,000 to 39,000 amperes per square meter is maintained on the surface of said cathode.

4. A process as defined in claim 1, wherein said chloride salt of an alkali metal is sodium chloride.

5. A process as defined in claim 4, wherein the concentration of sodium ions is at least about 2 grams per liter and the concentration of chloride ions is at least about 5 grams per liter.

6. A process as defined in claim 1, wherein the pH of said electrolyte is about 2.5 to 5.5, and following electrolysis said electrolyte has a pH of about 3.8 to 4.2;

and the pH is thereafter adjusted into the range of about 4.5 to 5.0 to provide a precipitate of at least one metal from the group consisting of cobalt, iron, arsenic and lead.

5 7. A process as defined in claim 1, wherein said electrolyte is oxidized to a concentration equivalent to 0.05 to 1.0 grams per liter of chlorine.

8. A process as defined in claim 1, wherein said electrolyte is subject to said current for about 2 minutes to about 20 minutes.

10 9. A process as defined in claim 1, wherein said equivalent chlorine is reacted with said impurity for a time period of about 20 minutes to about 2 hours.

15 10. A process as defined in claim 1, wherein said anode is an insoluble material resistant to corrosion in acid solution.

11. A process as defined in claim 1, wherein said cathode is a steel.

12. A process as defined in claim 1, wherein said electrolyte is agitated to prevent said metal hydroxide from settling.

13. A process for removing at least one impurity from a group consisting of cobalt, iron, arsenic and lead from an aqueous, essentially copper-free, nickel-containing electrolyte which comprises: immersing at least one anode and at least one cathode into said electrolyte, said electrolyte containing a chloride salt of an alkali metal; applying current between said anode and said cathode for a time period sufficient to generate in said electrolyte an equivalent chlorine content of at least about 0.05 and up to about 0.2 gram per liter while maintaining a current density at said cathode at a level sufficient to prevent substantial deposition of metal at said cathode but sufficient to generate a metal hydroxide in the vicinity of said cathode; increasing the pH of said electrolyte into a range of about 3.8 to 4.2 whereby said equivalent chlorine produced reacts with at least one impurity from a group consisting of iron,

20 arsenic and lead present in said electrolyte to provide a precipitate containing said at least one impurity; separating said precipitate from said electrolyte; reapplying current between said anode and said cathode for a time period sufficient to generate in said electrolyte an equivalent chlorine content of at least about 0.4 gram per liter while maintaining a current density at said cathode at a level sufficient to prevent substantial deposition of metal at said cathode but sufficient to generate a metal hydroxide in the vicinity of said cathode;

25 30 increasing the pH of said electrolyte into a range of about 4.5 to 5.0 whereby said equivalent chlorine produced reacts with at least one impurity from a group consisting of cobalt, iron, arsenic and lead present in said electrolyte to provide a precipitate containing said at least one impurity; and separating said precipitate from said electrolyte.

35 40 45 increasing the pH of said electrolyte into a range of about 4.5 to 5.0 whereby said equivalent chlorine produced reacts with at least one impurity from a group consisting of cobalt, iron, arsenic and lead present in said electrolyte to provide a precipitate containing said at least one impurity; and separating said precipitate from said electrolyte.

50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130

UNITED STATES PATENT OFFICE  
CERTIFICATE OF CORRECTION

PATENT NO. : 3,983,018

DATED : September 28, 1976

INVENTOR(S) : GYULA JOHN BORBELY, ALEXANDER ILLIS, & BERNARDUS  
JACOBUS BRANDT

It is certified that error appears in the above-identified patent and that said Letters Patent  
are hereby corrected as shown below:

In column 9, in Table VII, under the heading  
"chlorine", the number "0.085" should be "0.85".  
gpl

Signed and Sealed this  
Twenty-second Day of February 1977

[SEAL]

Attest:

**RUTH C. MASON**  
*Attesting Officer*

**C. MARSHALL DANN**  
*Commissioner of Patents and Trademarks*